

Sept. 6, 1960

R. S. DEAN

2,951,795

## PRODUCTION OF POLYVALENT METALS

Original Filed March 20, 1957



 INVENTOR  
Reginald S. Dean,

BY Pierce, Scheffler & Parker

his ATTORNEYS

# United States Patent Office

2,951,795

Patented Sept. 6, 1960

1

2,951,795

## PRODUCTION OF POLYVALENT METALS

Reginald S. Dean, Hyattsville, Md., assignor to Chicago Development Corporation, Riverdale, Md., a corporation of Delaware

Continuation of application Ser. No. 647,206, Mar. 20, 1957. This application June 9, 1958, Ser. No. 740,865

6 Claims. (Cl. 204—64)

This is a continuation of my application Serial No. 647,206, filed March 20, 1957, now abandoned.

This invention relates to the production of pure polyvalent metals of groups IV-B, V-B and VI-B of the periodic system, in coarse crystalline form.

It is known that coarse crystals of these metals are produced by passing a direct current between two inert electrodes in a molten bath consisting of alkalinous chlorides having dissolved therein chlorides of the polyvalent metal to be produced and also a significant amount of alkalinous metal. It is necessary for the continued operation of such baths that a means of maintaining the content of polyvalent metal chloride be provided. For this purpose, comminuted or particulate metal is provided in the electrolyte around the inert anode providing what is sometimes termed a disperse soluble anode. This comminuted material dissolves to maintain the bath.

This manner of proceeding to make coarse crystals of titanium has been fully described in a technical paper by the applicant entitled, "Electrolytic Titanium," published by the Chicago Development Corporation, January 1957.

It has also been known to produce particulate titanium dispersed in fused alkalinous chloride baths by sodium reduction and by passing a direct current through such baths, as for example, in British Patent No. 678,807, dated May 11, 1951, to Shawinigan Water and Power Company. In such procedures, it has been necessary to dissolve the salt bath from the particulate titanium dispersed in it before proceeding with further treatment of the metal. The dispersion of particulate metal in the salt has found no use per se. In fact, the effort of most workers in this field has been to cause the particles to grow in size and thus break up the dispersion.

In this invention, I make use of the dispersion as such and desire to have it as permanent as possible. Since some settling may unavoidably take place, I provide a stirrer in the cell and make provision to remove and recirculate any larger particles which may settle.

The replenishment of the electrolyte by a "disperse anode" is essentially different from normal electrorefining in which the direct electrical contact is made with the material to be dissolved. To use a "disperse anode," it is necessary to have an electrolyte in which the disperse particles dissolve chemically but only to an equilibrium amount; the change in electrolyte composition so brought about is then reversed by the electrochemical action at the anode. In this way the electrolyte is maintained.

The bobbin of the ordinary dry cell is a typical example of a disperse electrode.  $MnO_2$  surrounding the real graphite cathode quickly saturates the Leclanché electrolyte with  $Mn^{IV}$  ions but cathodic action reduces the dissolved  $Mn^{IV}$  so that more  $MnO_2$  can be dissolved. In this way,  $MnO_2$  acts as an electrode material although not actually connected in the circuit.

I have so far illustrated the type of dispersion I use with dispersions of titanium metal. Dispersions of the

2

polyvalent metals of group IV-B, V-B and VI-B may be produced by analogous procedures. In addition, certain metallic compounds may be produced dispersed in salt and these dispersions may be used to maintain the bath. For example, the metallic compound  $ZrCl$  may be produced dispersed in a salt melt by the action of  $ZrCl_4$  on Zr metal in a melt of sodium chloride.

This invention, then, consists in taking the particulate metal or electrically conductive metallic compound in a salt bath, partially removing the salt by settling of the metal, adding the dispersion so enriched in metal, either before or after solidification, to an electrolytic cell in which the dispersion of metal or metallic compound provides the "disperse soluble anode."

It will be clear that some of the salt bath must be removed with the crystals attached to the cathode so that the volume of bath will be maintained by adding the particulate metal admixed with salt. By suitable adjustment of current with respect to active anode surface, the content of polyvalent metal chloride in the bath may be maintained constant.

Having now described the general features of my invention, I will illustrate it by specific examples.

### Example I

In this example, I use as the source of the polyvalent metal titanium dioxide. I reduce this oxide with carbon at 800° C. to increase its ease of chlorination. I form this reduced titanium oxide approximating  $Ti_3O_5$  in composition into pellets using an amount of tar so that on heating I obtain pellets containing the stoichiometric equivalent of oxygen and carbon to form oxides of carbon at 850° C. I place these pellets in a cell having a graphite anode in the midst of said pellets; an electrolyte of fused sodium chloride is provided the cell. The cell with graphite anode *a* and pellets *b* is shown in Figure 1. The cell is also provided with a steel cathode *c* as shown. When a direct current is passed through the cell,  $TiCl_4$  is formed in the anode zone and passes through the molten electrolyte to the cathode zone where particulate *Ti* is formed and falls to the bottom of the cell where it is removed through the gate *d* with about 25% of its weight as fused salt into a second cell having an iron anode *e* and an iron cathode *f* and a stirring device *g* to maintain the particulate titanium in suspension. The second cell is provided with an electrolyte of molten sodium chloride in which is dissolved from 3-8% *Ti* as chloride and from 1-3% sodium. When a direct current is passed through the second cell, the particulate titanium is dissolved and a salt layer with finely dispersed titanium crystals formed on the cathode, this is surrounded on further passage of the direct current with coarse crystal intergrowths of pure titanium frangibly attached by the viscous salt layer to the cathode. From time to time the cathode is lifted above the level of the electrolyte and into gas-tight draining and cooling chamber *h* which surmounts and communicates with the second cell, the chamber being closable by means of valve *i* and being operable at its top by means of closure member *j*, cooled out of contact with air and the crystal intergrowths removed and washed with dilute acid. The preformed cathode is returned to the bath which is replenished from time to time by additions of particulate titanium and fused salt from the first cell. The washed crystals show less than .02% oxygen and no other determinable impurities.

At *k* is indicated a conventional gas lock for use in introducing pellets of  $TiCl_3$  plus carbon into the space surrounding anode *a*, and *l* is indicated a conventional lock for use in removing anode residue which may have accumulated adjacent the lower end of anode *a*. The bottom of the second cell preferably is downwardly sloped, as

shown at *m*, to provide a sump space *n*, from the lowermost part of which latter extends a draw-off conduit *o*, provided with a draw-off valve *p*, for the occasional withdrawal of bath material and settled out solid particles.

*Example II*

In this example, I use as the source of the polyvalent metal chromite  $\text{FeO}\text{Cr}_2\text{O}_3$ . I mix powdered chromite with carbon in sufficient amount to form  $\text{CO}_2$  from all oxygen present and form into pellets. I chlorinate these pellets to form  $\text{CrCl}_3$  and  $\text{FeCl}_3$  which I condense as sublimes. I add this sublimate to molten sodium chloride alternately with small amounts of sodium to form a particulate metal having a ratio of chromium to iron of about 2-1. This particulate metal settles in the molten  $\text{NaCl}$  and the enriched mixture of metal particles and salt is withdrawn and is added to an electrolytic cell having an electrolyte of  $\text{NaCl}$  having dissolved therein about 5% Cr, mostly as  $\text{CrCl}_2$  with a little  $\text{CrCl}_3$  and about 1% sodium, an iron anode and an iron cathode. A direct current is passed through the cell causing the chromium to dissolve from the particulate metal and form chromium crystals attached to the cathode. The iron particles remain unattacked in the bath and from time to time the bath is withdrawn, cooled and pulverized and the iron removed magnetically and the purified salt returned to the cell.

All of the operations described are carried out in the absence of air.

The chromium crystals are washed with dilute acid and on analysis show 99.9% chromium and less than .01% oxygen.

*Example III*

In this example, I use zirconium carbide as the source of the polyvalent metal and chlorinate it to produce  $\text{ZrCl}_4$ . I add this to the cathode compartment of a diaphragm cell containing an electrolyte of 65%  $\text{SrCl}_2$ , 35%  $\text{NaCl}$  at 600° C. The  $\text{ZrCl}_4$  is added at the rate at which it is reduced to metal by the alkalinous metal formed at an iron cathode. A graphite anode is provided in the anode compartment and the chlorine is recovered and used to chlorinate the zirconium carbide. Particulate zirconium is formed in the cathode compartment of the cell and settles to the bottom from which it is recovered with about 20% of the fused salt bath. The mixture of bath and particulate zirconium is added to an electrolytic cell having an iron cathode and anode, an electrolyte of 65%  $\text{SrCl}_2$ , 35%  $\text{NaCl}$  in which is dissolved 10% zirconium as a mixture of  $\text{ZrCl}_2$  and  $\text{ZrCl}_3$  having an average valence of 2.3 and 3% alkalinous metal. The temperature of electrolysis is 600° C. and zirconium crystals of high purity are formed attached to the cathode. All of the operations described are carried out in an argon atmosphere.

The zirconium crystals are washed with dilute acid and analyze less than .01% oxygen and no determinable amounts of other impurities.

*Example IV*

In this example, I take finely divided metallic zirconium in excess and heat it in an inert atmosphere with fused sodium chloride containing  $\text{ZrCl}_4$  under pressure at 825° C. After heating for 100 hours, the chlorine of the  $\text{ZrCl}_4$  has been converted entirely to  $\text{ZrCl}$  which is found in dispersion in the salt as fine flaky particles. I feed this dispersion continuously into a cell like that of *g* in the drawing and pass a direct current until the bath contains 10% suspended  $\text{ZrCl}$  through the bath at 200 amperes per sq. ft. on the cathode. Crystalline zirconium is formed on the cathode and the dispersion of  $\text{ZrCl}$  is then fed at the rate necessary to maintain the zirconium content of the bath. The bath contains 3% zirconium dissolved as chloride, average valence 2.1 and .5% dissolved metallic sodium.

I claim:

1. In a process for depositing a metal selected from a first group consisting of titanium, zirconium and chromium from an electrolyte of at least one fused chloride of at least one second group metal selected from the group consisting of alkali and alkaline earth metals and dissolved therein 2-10% of a chloride of the first group metal and .1-3% of a metal selected from said second group consisting of alkali metals and alkaline earth metals by passing a current through said electrolyte between two inert electrodes whereby to form a layer of finely dispersed crystals of the metal of the first group in a salt layer on the cathode, the improvement which consists in continuing the passage of current while replenishing the electrolyte with the metal to be deposited by the addition to the electrolyte of a dispersion of particles of a material selected from a group consisting of (a) the metal to be deposited and (b) an electrically conducting metallic compound of zirconium and chlorine, in a chloride of a metal of the second group, whereby to obtain the metal of the first group in the form of coarse crystal intergrowths adherent to the salt layer on the cathode.
2. In a process for depositing a metal selected from a first group consisting of titanium, zirconium and chromium from an electrolyte of at least one fused chloride of at least one second group metal selected from the group consisting of alkali and alkaline earth metals and dissolved therein 2-10% of a chloride of the first group metal and .1-3% of a metal selected from said second group consisting of alkali metals and alkaline earth metals by passing a current through said electrolyte between two inert electrodes whereby to form a layer of finely dispersed crystals of the metal of the first group in a salt layer on the cathode, the improvement which consists in continuing the passage of current while replenishing the electrolyte with the metal to be deposited by the addition to the electrolyte of a dispersion of particles of the metal to be deposited in a chloride of a metal of the second group, whereby to obtain the metal of the first group in the form of coarse crystal intergrowths adherent to the salt layer on the cathode.
3. In a process of depositing zirconium from an electrolyte of at least one fused chloride of at least one reducing metal of the group consisting of alkali and alkaline earth metals and dissolved therein 2-10% of a chloride of zirconium and 0.1-3.0% of at least one of said reducing metals by passing a current through said electrolyte between two inert electrodes whereby to form a layer of zirconium crystals in a salt layer on the cathode, the improvement which consists in continuing the passage of current while replenishing the electrolyte with zirconium by the addition to the electrolyte of a dispersion of particles of  $\text{ZrCl}$  in sodium chloride, whereby to obtain zirconium in the form of coarse crystal intergrowths adherent to the salt layer on the cathode.
4. In a process of depositing zirconium from an electrolyte of at least one fused chloride of at least one reducing metal of the group consisting of alkali and alkaline earth metals and dissolved therein 2-10% of a chloride of zirconium and 0.1-3.0% of at least one of said reducing metals by passing a current through said electrolyte between two inert electrodes whereby to form a layer of zirconium crystals in a salt layer on the cathode, the improvement which consists in continuing the passage of current while replenishing the electrolyte with zirconium by the addition to the electrolyte of a dispersion of particles of zirconium metal in sodium chloride, whereby to obtain zirconium in the form of coarse crystal intergrowths adherent to the salt layer on the cathode.
5. In a process of depositing titanium from an electrolyte of at least one fused chloride of at least one reducing metal of the group consisting of alkali and alkaline earth metals and dissolved therein 2-10% of a chloride of titanium and 0.1-3.0% of at least one of said reducing

metals by passing a current through said electrolyte between two inert electrodes whereby to form a layer of titanium crystals in a salt layer on the cathode, the improvement which consists in continuing the passage of current while replenishing the electrolyte with titanium by the addition to the electrolyte of a dispersion of particles of titanium metal in sodium chloride, whereby to obtain titanium in the form of coarse crystal intergrowths adherent to the salt layer on the cathode.

6. In a process of depositing chromium from an electrolyte of at least one fused chloride of at least one reducing metal of the group consisting of alkali and alkaline earth metals and dissolved therein 2-10% of a chloride of chromium and 0.1-3.0% of at least one of said reducing metals by passing a current through said electrolyte between two inert electrodes whereby to form a layer of chromium crystals in a salt layer on the

cathode, the improvement which consists in continuing the passage of current while replenishing the electrolyte with chromium by the addition to the electrolyte of a dispersion of particles of chromium metal in sodium chloride, whereby to obtain chromium in the form of coarse crystal intergrowths adherent to the salt layer on the cathode.

References Cited in the file of this patent

UNITED STATES PATENTS

|           |                |               |
|-----------|----------------|---------------|
| 2,734,856 | Schultz et al. | Feb. 14, 1956 |
| 2,748,073 | Mellgren       | May 29, 1956  |
| 2,760,930 | Alpert et al.  | Aug. 28, 1956 |
| 2,817,631 | Gullett        | Dec. 24, 1957 |

FOREIGN PATENTS

|         |               |               |
|---------|---------------|---------------|
| 682,919 | Great Britain | Nov. 19, 1952 |
|---------|---------------|---------------|